

1

2,767,143

LUBRICATING COMPOSITIONS CONTAINING  
METAL DERIVATIVES OF 1,3-BIS(HYDROXY-ARALKYL)-2-IMIDAZOLIDINETHIONES

James M. Caffrey, Jr., Beacon, and Herman D. Kluge and John E. Tessieri, Wappingers Falls, N. Y., assignors to The Texas Company, New York, N. Y., a corporation of Delaware

No Drawing. Application June 5, 1952,  
Serial No. 291,994

6 Claims. (Cl. 252—42.7)

The present invention relates to improved lubricating compositions, and more particularly to lubricating compositions containing metal derivatives of substituted cyclic thioureas.

It is common practice to add to mineral lubricating oils small amounts of so-called "detergent" compounds of various types, which have the property either of reducing the formation of gums and sludges, normally occurring as a result of the oxidative or other deterioration of the oil under service conditions, or of dispersing and altering the character of any gums and sludges formed so as to reduce the formation of varnish-like deposits upon the lubricated engine parts.

Among the compounds which have been proposed as lubricating oil additives of the detergent type are the metal derivatives of condensation products obtained by interreacting hydroxyaromatic compounds with aldehydes and with amines, including polyamines containing at least two reactive, i. e., primary or secondary, amine groups, as disclosed in U. S. 2,353,491. The hydroxy metal and alkoxy metal derivatives of such condensation products, disclosed in the copending application of H. D. Kluge and F. W. Moore, Serial Number 287,266, now Patent No. 2,725,357, filed May 10, 1952, have been found to be particularly effective for this purpose. However, the above compounds have also been found to exert a pronounced pro-oxidant effect upon lubricating oils at elevated temperatures, which results in an objectionable increase in the acidity of the oils during use. Sulfurization of these compounds by reacting them with sulfur or a sulfur halide, as disclosed in U. S. 2,459,114, accomplishes some improvement in their pro-oxidant activity, but also largely destroys their detergent properties.

This invention is based upon the discovery that very superior detergent-type additives for mineral lubricating oils are obtained by reacting certain compounds of the above type with carbon disulfide. We have found that the sulfur-containing compounds thus obtained have excellent detergency characteristics equivalent to the corresponding unsulfurized compounds, but without the objectionable pro-oxidant characteristics of the latter.

The novel lubricating oil additives of this invention are metal derivatives of reaction products obtained by first interreacting a hydroxyaromatic compound with an aldehyde and with a polyamine containing two primary amine groups separated by two carbon atoms, so as to form a condensation product, and then further reacting this condensation product with carbon disulfide. The metal derivatives include the normal metal salts and the hydroxy-metal and alkoxy-metal derivatives. Preferably, the compound contains at least one aliphatic hydrocarbon group of sufficient chain length to impart oil-solubility.

Typical hydroxyaromatic compounds which may be employed in forming the condensation product include phenol, diethyl phenol, pentacosyl phenol, alpha- and beta-naphthol, octadecyl alpha- and beta-naphthol, catechol, benzylphenol, chlorophenol, hydroquinone, phe-

2

nol resins, and the like. The preferred compounds of this class are alkyl hydroxyaromatic compounds containing at least one aliphatic hydrocarbon substituent group of from about 5 to 30 carbon atoms. The terms "alkyl hydroxyaromatic," "alkyl phenol," etc., are used for convenience in the specification and claims to mean compounds containing one or more aliphatic hydrocarbon groups, which may be either saturated or unsaturated in character.

10 Aldehydes employed in forming the condensation product are preferably aliphatic aldehydes such as formaldehyde, acetaldehyde, butyraldehyde, furfuraldehyde, etc., although aromatic aldehydes such as benzaldehyde, toluic aldehyde, etc., may also be employed if desired.

15 The aldehydes may contain substituent groups such as hydrocarbon groups, alkoxy groups, nitro groups, halogens, etc., insofar as these do not interfere in the condensation reaction.

The polyamine employed in forming the condensation product is preferably ethylene diamine, or a hydrocarbon compound which may be regarded as a derivative of ethylene diamine, preferably such derivatives wherein not more than one hydrogen on each methylene group is substituted by a hydrocarbon group. As examples of such compounds may be mentioned 1,2-propylene diamine, 1,2-butylene diamine, 2,3-butylene diamine and phenyl ethylene diamine. Aromatic compounds containing adjacent primary amine groups, such as ortho-phenylene diamine, may also be employed. The amine may contain various substituent groups as discussed above in connection with the aldehyde reactant.

The condensation reaction is suitably carried out by heating the reactants together at a moderately elevated temperature, such as a temperature in the range of about 100–200° F., in the presence or absence of a solvent. The reactants are preferably employed in approximately equivalent reacting proportions, i. e., about equimolar proportions of hydroxyaromatic compound and of aldehyde with about one half mole of the amine.

40 The product obtained by the above condensation reaction appears to consist predominantly of N,N'-bis(hydroxy aralkyl) diamines, with smaller amounts of both higher and lower condensation products. Investigations by Donia et al. (Journal of Organic Chemistry, 45 vol. 14, pages 946–951 (1949)) have indicated that compounds of this character, containing an ethylene diamine group, react with carbon disulfide in two stages to form cyclic thioureas, as follows:



The above reaction with carbon disulfide is carried out by mixing the reactants and then heating at a moderately elevated temperature, suitably in the range of from about 100° F. to about 300° F., in the presence or absence of a mild oxidizing agent such as iodine. Equimolar pro-

portions of the diamine condensation product and carbon disulfide may be employed in the reaction, but preferably an excess of carbon disulfide is employed, amounting to at least a two-fold excess over the amount theoretically required.

Metal derivatives of the reaction products prepared as described above are obtained by replacing the hydroxyl hydrogens of the hydroxyaryl groups with their equivalent of a metal. Any metal in general may be employed for this purpose which can be suitably reacted to form the oxyaryl derivatives, such as for example sodium, potassium, magnesium, calcium, barium, manganese, iron, tin, copper, cobalt, and so forth. Because of the generally superior detergency characteristics of compounds of alkaline earth metals and zinc, the metal is preferably chosen from this group. With particular advantage, where the compounds are to be employed as additives where the character of the combustion chamber deposits is an important consideration, the metal is chosen from the group consisting of magnesium and zinc. For regular heavy duty motor oils, however, the heavier metals such as calcium and barium may be suitably employed. As discussed hereinabove, the derivatives may be a normal metal salt, i. e., wherein the metal is connected only to one or more oxyaryl groups of the amine condensation product, or it may be a hydroxy-metal or alkoxy-metal derivative, wherein the alkoxy group contains from 1 to 5 carbon atoms, as disclosed in the aforementioned application of Kluge et al.

The metal derivative may be prepared conveniently by the method comprising reacting the amine condensation product with a metal methylate or other lower alcoholate of a metal, employing approximately equal molar proportions to obtain the normal metal salt, and employing at least two moles of metal alcoholate for each mole of the amine condensation product to obtain the alkoxy-metal derivative. The hydroxy-metal derivatives may be readily obtained by hydrolysis of the alkoxy-metal derivatives obtained as described above. The normal metal salts may also be obtained by various other well-known reactions, such as by reacting the amine condensation product with metal hydroxide. Conversion to the metal derivatives may be carried out either before or after the amine condensation product is reacted with carbon disulfide.

The novel additives of this invention may be employed in lubricating oils in various amounts, ranging from very small amounts up to amounts representing the limits of their solubilities, depending upon the effect desired. For ordinary purposes, they are suitably employed in amounts within the range of from about 0.1 to about 5.0 percent by weight, and preferably within the range of from about 0.25 to about 2.0 percent by weight of the lubricating composition. In addition to these compounds, other lubricating oil additives may also be employed if desired such as extreme pressure agents, pour depressants, corrosion inhibitors, and so forth.

In order to more fully disclose the invention, the preparation of a typical compound of this novel class of lubricating oil additives is described in detail in the following example.

#### EXAMPLE 1

A condensation product was prepared by reacting an alkyl phenol with formaldehyde and with ethylene diamine. The alkyl phenol was a purchased product having a hydroxyl number of 128 and a molecular weight of 440, indicating that it consisted chiefly of an alkylated phenol containing an average of 25 carbon atoms in the alkyl group. In carrying out the condensation, 2640 grams (6 moles) of the alkyl phenol, 262 grams (3 moles) of ethylene diamine and 4.5 liters of ethyl alcohol were introduced into a flask and 525 grams (6 moles plus 5 percent excess) of formaldehyde in the form of a 36 percent solution were added slowly over a 2 hour period.

The reaction mixture was then heated under reflux for 8 hours. The reaction product was recovered by cooling the reaction mass to room temperature, dissolving in ether and washing the ether solution first with a saturated sodium chloride solution and then with water until neutral to Brilliant Yellow. The ether was then stripped off, with toluene added as a make-up solvent until the toluene boiling point was reached, and the toluene finally stripped off under a vacuum. The product thus obtained contained 2.51 percent of nitrogen, as compared to the theoretical value of 2.91 percent for the compound



N,N'-bis(2-hydroxy-alkyl (C<sub>25</sub>) benzyl)-1,2-diamino ethane

0.3 mole of the above condensation product in the form of a toluene solution were mixed with 76 grams (1 mole) of carbon disulfide and the mixture refluxed for 50 hours. 100 grams of a 300 SAE grade lubricating oil were then added, the solution filtered and stripped at 270-300° F. for one hour under a vacuum of 5 millimeters of mercury to remove the solvent. 305 grams of product were recovered, which analyzed 3.1 percent of sulfur, as compared with the theoretical value of 2.4 percent (calculated on the basis of a 75.3 percent concentrate) for the compound



1,3-bis-(2-hydroxy-alkyl (C<sub>25</sub>) benzyl)-2-imidazolidinethione

The product therefore appeared to be predominantly the cyclic thiourea shown above in admixture with a small amount of the dithiocarbamic acid inner salt first formed in the reaction (Equation I).

The normal magnesium salt of the above reaction product was prepared in the following manner: 302 grams of the lubricating oil solution, containing approximately 0.29 mole of the reaction product, were mixed with 224 milliliters of a 0.31 molar methanol solution of magnesium methylate (0.29 mole) and the mixture allowed to react. After the reaction was completed, a 300 SAE grade lubricating oil was added, sufficient to form a 50 percent concentrate of the reaction product, and the solvent stripped off at 90° C. for 2.5 hours under a vacuum of 5 millimeters of mercury. The solution thus obtained analyzed 5.85 percent ash and 1.16 percent magnesium, as compared with the theoretical values of 5.81 percent and 1.16 percent, respectively, calculated for a 50 percent solution of the normal magnesium salt of 1,3-bis-(2-hydroxy-alkyl(C<sub>25</sub>)benzyl)-2-imidazolidinethione.

The superior properties of the above compound as a lubricating oil additive of the detergent type in comparison with the corresponding compounds of the prior art are shown in Tables I and II below.

All of the additives shown in the tables were derived from condensation products obtained by interreacting alkyl phenols with formaldehyde and with ethylene diamine in the manner described in Example 1. The normal magnesium salt was obtained by reaction of such a condensation product with magnesium methylate in approximately equimolar proportions, as described in Example 1. The normal zinc salt was obtained by first forming the sodium salt by reaction of the condensation product with sodium butylate, and then reacting this sodium salt with zinc chloride. The normal barium salt was obtained by reacting the condensation product with

barium hydroxide. The methoxy-magnesium derivatives were obtained by reacting the condensation product with magnesium methylate, employing two mol proportions of magnesium methylate for each mol proportion of condensation product, as described in the aforementioned application of Kluge et al. The disulfurized magnesium derivative was obtained by reacting the condensation product with sulfur monochloride, employing approximately equimolar proportions of the two reactants in pentane solution, and then converting the sulfurized product obtained to the magnesium derivative as described above. In preparing the mono-sulfurized compounds the disulfurized condensation product, obtained as described above, was treated with sodium sulfite in sodium hydroxide solution, employing approximately equimolar proportions of the two reactants. The sulfurized compound resulting from this treatment was then converted to the magnesium and to the methoxy-magnesium derivatives as described above. The above compounds were employed in the form of 1 percent solutions in the base oil, which was a refined paraffinic distillate lubricating oil of medium viscosity. For convenience, the compounds are referred to in the tables as derivatives of the *N,N'*-bis(hydroxy-alkyl-benzyl)-1,2-diamino ethanes, which are thought to comprise the chief component of the condensation products.

The oxidation test of Table I is an uncatalyzed oxidation test which is primarily useful in indicating the oxidation directing properties of lubricating oil additives, that is, whether they are pro-oxidants or anti-oxidants. The apparatus employed in this test is a closed system through which oxygen is circulated, comprising an oxidation tube, a scrubber for removing volatile acids, water and carbon dioxide, and a calibrated burette for measuring the oxygen consumption. The oxidation tube is immersed in an oil bath maintained at  $339 \pm 1$ ° F. In carrying out the test, 21 grams of the test oil are placed in the oxidation tube, air is displaced from the system and oxygen (about 98.3 percent purity) is circulated at a constant rate of 2.2 liters per hour for the period of the test, ordinarily for 40 hours. As the oxygen is consumed, thereby diminishing the pressure in the closed system, valves automatically open to permit oil from a reservoir to drain into the burette to reestablish the pressure, and the amount of oxygen consumed is read directly from the oil level in the burette. A weighed glass slide is suspended in the test oil during the test, and at the end of the test the slide is removed, washed with pentane, dried and reweighed to determine the amount of varnish deposition.

Table I.—Oxidation test

| Additive                                                                                                                                     | Varnish, mg. | Oxygen absorption, millimoles/hours | N. N. Used Oil |
|----------------------------------------------------------------------------------------------------------------------------------------------|--------------|-------------------------------------|----------------|
| None (base oil)                                                                                                                              | 10.8         | 21/40                               | 3.8            |
| 1% of Ba salt of <i>N,N'</i> -bis(hydroxy-alkyl ( $C_{22}$ )benzyl)-1,2-diamino ethane                                                       | 1.8          | 58/17                               | 15.0           |
| 1% of Zn salt of <i>N,N'</i> -bis(hydroxy-alkyl ( $C_{22}$ )benzyl)-1,2-diamino ethane                                                       | 4.2          | 55/20                               | 14.9           |
| 1% of Mg salt of <i>N,N'</i> -bis(hydroxy-alkyl ( $C_{22}$ )benzyl)-1,2-diamino ethane                                                       | 1.1          | 54/15                               | 12.4           |
| 1% of Mg salt of sulfurized <i>N,N'</i> -bis(hydroxy-alkyl ( $C_{22}$ )benzyl)-1,2-diamino ethane                                            | 23.7         | 54/38                               | 8.9            |
| 1% of Mg salt of disulfurized <i>N,N'</i> -bis(hydroxy-alkyl ( $C_{22}$ )benzyl)-1,2-diamino ethane                                          | 11.0         | 26/40                               | 3.1            |
| 1% of methoxy-Mg derivative of <i>N,N'</i> -bis(hydroxy-alkyl ( $C_{19}$ )benzyl)-1,2-diamino ethane                                         | 0.0          | 55/13                               | 12.3           |
| 1% of methoxy-Mg derivative of sulfurized <i>N,N'</i> -bis(hydroxy-alkyl ( $C_{22}$ )benzyl)-1,2-diamino ethane                              | 6.7          | 55/29                               | 12.1           |
| 1% of Mg salt of reaction product of <i>N,N'</i> -bis(hydroxy-alkyl ( $C_{22}$ )benzyl)-1,2-diamino ethane with carbon disulfide (Example 1) | 4.7          | 23/40                               | 3.9            |

Table II below also shows the detergency characteristics under conditions simulating those encountered in crankcase lubrication of a lubricating oil containing the compound of Example 1 in comparison with oils containing the corresponding unsulfurized compound and the sulfurized compounds of the prior art. The Toettcher varnish test and the high temperature deposits test of the table are bench tests which have been found to correlate well with the lacquer forming and the oil ring sticking characteristics of a cylinder oil in actual service. In the Toettcher varnish test, a weighed glass cylinder is immersed in a sample of the test oil maintained at 350° F. and agitated by a centrifugal mixer. Copper baffles are also immersed in the test oil to act as oxidation catalysts. After 13 hours the test is terminated and the glass cylinder removed, washed with gasoline, dried and reweighed. The amount of varnish deposited on the cylinder is the difference between the initial and final weights of the cylinder. The neutralization number of the used oil is also determined. The high temperature deposits test is carried out by repeatedly dipping an aluminum cylinder one inch in diameter and three inches long into a beaker containing a sample of the test oil maintained at 525° F. for a period of 20 hours. The test specimen is then washed with pentane and dried, and the weight of deposits found by the increase in weight. The test specimen is then brushed to remove loose deposits and reweighed to determine the amount of varnish-like deposits. A lubricating oil of the same type as that employed in the oxidation test of Table I was employed in these tests.

Table II.—Detergency tests

| Additive                                                                                                                                     | Toettcher Varnish Test, 350° F. |                | High Temperature Deposits Test, 525° F. |          |
|----------------------------------------------------------------------------------------------------------------------------------------------|---------------------------------|----------------|-----------------------------------------|----------|
|                                                                                                                                              | Weight of deposits, mg.         | N. N. Used oil | Weight of deposits, mg.                 |          |
|                                                                                                                                              |                                 |                | Total                                   | Adherent |
| None (base oil)                                                                                                                              | 15.2                            | 6.0            | 452                                     | 326      |
| 1% of Mg salt of <i>N,N'</i> -bis(hydroxy-alkyl ( $C_{22}$ )benzyl)-1,2-diamino ethane                                                       | 3.7                             | 12.5           | 115                                     | 15       |
| 1% of Mg salt of sulfurized <i>N,N'</i> -bis(hydroxy-alkyl ( $C_{22}$ )benzyl)-1,2-diamino ethane                                            | 14.8                            | 8.1            | 34                                      | 14       |
| 1% of Mg salt of disulfurized <i>N,N'</i> -bis(hydroxy-alkyl ( $C_{22}$ )benzyl)-1,2-diamino ethane                                          | 12.7                            | 6.5            | 106                                     | 83       |
| 1% of Mg salt of reaction product of <i>N,N'</i> -bis(hydroxy-alkyl ( $C_{22}$ )benzyl)-1,2-diamino ethane with carbon disulfide (Example 1) | 2.0                             | 3.9            | 79                                      | 29       |

As shown by the above tables, the compound of this invention had excellent detergency characteristics fully equivalent to those of the corresponding unsulfurized metal derivative in a mineral lubricating oil, and was substantially without effect upon the oxygen absorption or acidity increase of the oil. On the other hand, all of the corresponding unsulfurized compounds of the prior art tested had a strong pro-oxidant effect, and their sulfurized derivatives of the prior art were entirely, or almost entirely, lacking in detergent effect.

Obviously many modifications and variations of the invention, as hereinbefore set forth, may be made without departing from the spirit and scope thereof and, therefore, only such limitations should be imposed as are indicated in the appended claims.

We claim:

1. A lubricating composition comprising a mineral lubricating oil containing about 0.1 to about 5.0 percent by weight of a metal derivative of the reaction product at an elevated temperature of carbon disulfide with a condensation product of one mol equivalent of a hydroxyaromatic compound with about one mol equivalent of an aldehyde and at least about one half mol equiva-

lent of an amine compound containing two primary amine groups separated by two carbon atoms, said metal derivative having the hydroxyl hydrogens of the said reaction product replaced by a member of the group consisting of metals, metal hydroxides, and metal alkoxides containing from 1 to 5 carbon atoms.

2. A lubricating composition comprising a mineral lubricating oil containing about 0.1 to about 5.0 percent by weight of a metal derivative of the reaction product at an elevated temperature of carbon disulfide with a condensation product of one mol equivalent of a hydroxyaromatic compound, containing an alkyl substituent group of sufficient chain length to impart oil-solubility to the final product, with about one mol equivalent of an aliphatic aldehyde and at least about one half mol equivalent of an aliphatic amine containing two primary amine groups separated by two carbon atoms, said metal derivative having the hydroxyl hydrogens of the said reaction product replaced by a member of the group consisting of metals, metal hydroxides, and metal alkoxides containing from 1 to 5 carbon atoms.

3. A lubricating composition comprising a mineral lu-

5

10

15

20

bricating oil containing about 0.1 to about 5.0 percent by weight of a metal derivative of the reaction product at an elevated temperature of carbon disulfide with a condensation product of one mol equivalent of an alkyl phenol, in which an alkyl substituent on the benzene nucleus contains from about 5 to about 30 carbon atoms, with about one mol equivalent of formaldehyde and at least about one half mol equivalent of ethylene diamine, said metal derivative having the hydroxyl hydrogens of the said reaction product replaced by a member of the group consisting of metals, metal hydroxides, and metal alkoxides containing from 1 to 5 carbon atoms.

4. Claim 3 wherein the metal is a member of the group consisting of alkaline earth metals and zinc.

5. Claim 3 wherein the metal is magnesium.

6. Claim 3 wherein the metal is zinc.

References Cited in the file of this patent

UNITED STATES PATENTS

2,353,491 Oberright \_\_\_\_\_ July 11, 1944  
2,596,742 Vaughn et al. \_\_\_\_\_ May 13, 1952